

C. W. DAVIS.

COMPOUND METALLIC ARTICLE.

APPLICATION FILED FEB. 15, 1913. RENEWED NOV. 24, 1913.

1,101,729.

Patented June 30, 1914

FIG.1.



FIG.2.



FIG.3.



WITNESSES:

J. Herbert Bradley.  
Francis J. Tomanow

INVENTOR

Charles W. Davis  
by Christy and Christy  
Atty's

# UNITED STATES PATENT OFFICE.

CHARLES W. DAVIS, OF EDGEWORTH, PENNSYLVANIA, ASSIGNOR TO STANDARD UNDERGROUND CABLE CO., OF PITTSBURGH, PENNSYLVANIA, A CORPORATION OF PENNSYLVANIA.

## COMPOUND METALLIC ARTICLE.

1,101,729.

Specification of Letters Patent. Patented June 30, 1914.

Application filed February 15, 1913, Serial No. 748,719. Renewed November 24, 1913. Serial No. 802,801.

To all whom it may concern:

Be it known that I, CHARLES W. DAVIS, residing at Edgeworth, in the county of Allegheny and State of Pennsylvania, a citizen 5 of the United States, have invented or discovered certain new and useful Improvements in Compound Metallic Articles, of which improvements the following is a specification.

10 My invention relates to improvements in the methods of forming compound metallic articles, and specifically to improvements in that method of formation which involves inclosing or incasing a body of one metal with 15 in an envelop of another metal, and elongating or extending a blank so compounded, the component bodies of metal being both of them, at the time when the blank is assembled, at temperatures below their melting 20 points.

While my invention is not limited to specific metals, nor to a specific article, I shall describe it in its application to the production of compound metallic wire having a 25 core of steel, and a covering of copper. This material is now commercially produced by a method which involves the surrounding of a core of steel with a sleeve of copper, both metals being in solid state, and in then 30 bringing the blank so compounded to rolling temperature, and rolling it to rod form, and subsequently drawing the rod to wire. It is a matter of first importance in this material that the union of the two metals, which 35 is effected in the early stages of the rolling operation, be most intimate, and it is apparent that the existence of an appreciable space between the adjacent surfaces of the copper and the steel, prior to that point in the operation where intimate union is effected, is 40 undesirable; or, stated in other words, it is desirable to bring the surfaces of the components into the closest possible contact in order to get the best results. It will be understood that in the specific case of copper 45 enveloping steel, the difficulty due to the presence of any space, or rather the problem of eliminating, so far as possible, the space between the surfaces, is aggravated by the 50 fact that the coefficients of expansion of these two metals are not alike, and that copper expands as it is heated more rapidly than does steel. The consequence is that though when the blank is assembled the 55 space interval between the adjacent surfaces

may be at a minimum, in the subsequent heating operation preparatory to rolling the space will necessarily be enlarged. It will be understood further, by those who are familiar with this industry, that inasmuch as 60 the rolling operation (under conditions now practised) involves the introduction of a blank circular in cross section to an initial roll pass which is rectangular in cross section, the first effect of rolling is to compress 65 the adjacent surfaces together at diametrically opposite points, and at the same time to cause or tend to cause the separation of the surfaces at intermediate points. It will be understood by those familiar with the 70 practice that, inasmuch as in succeeding roll passes the article under treatment is shifted by turning on its axis about 90°, there are successively produced strains which tend to open the interstices between the component 75 bodies, as well as strains which tend to close them, and it is a fact that gaps are at times produced. The presence of appreciable spaces between the adjacent surfaces of the components is undesirable, particularly 80 at the temperature of rolling, because the presence of oxid on the adjacent surfaces is inimical to intimate union, and because at the elevated temperature of rolling the metals are peculiarly liable to oxidation, and because the intrusion of air into such spaces as may exist is a cause which may produce oxidation. 85

My invention may be stated in general terms to consist of a method of forming 90 compound metallic bodies in which a core of relatively cold material is surrounded by a covering of relatively hot material, and the blank thus formed is subsequently brought to a temperature proper for reduction or 95 extension.

Specifically in case of copper-clad steel wire, my method is employed in inclosing the core of steel at relatively low temperature in a sleeve of copper at relatively 100 high temperature (both bodies of metal being at temperatures lower than the several melting points) and then subjecting the compound blank to the usual operations of reduction. In initially uniting the components, I may practise one or another of several expedients. For example, the existing practice is to properly prepare the steel core and the copper sleeve, and then to drive the sleeve over the core. In adapting my in- 105

vention to this procedure, I preferably employ a copper sleeve and a steel core of such relative sizes that while they may not be united when both are at normal atmospheric temperatures, the enlargement of the copper sleeve under a permissible increase of temperature will be sufficient to permit of assembling them by inserting the core within the sleeve. When the components have been properly prepared, I heat the copper sleeve (preferably in a non-oxidizing atmosphere) to a point lower than the melting point of the copper, but to a point at which it will be so enlarged as to permit the introduction within it of the previously prepared steel core, while the latter is at a lower and (as ordinarily will be the case) at substantially atmospheric temperature. I then bring the two bodies together, using if found desirable such appliances as are ordinarily employed in the existing practice. I then allow the temperature of the combined bodies to be equalized, that is to say, I either bring the whole to atmospheric temperature, or to substantially atmospheric temperature, or else I place the blank, formed by bringing the two bodies together, in the furnace where it is heated preparatory for rolling, and keep it there until core and sleeve are together brought to rolling temperature. Whether this equalization of temperature be by bringing the whole to atmospheric temperature, or by placing the blank in a furnace where the core will be heated until a uniform temperature with the sleeve, the effect will be the same, namely, to cause the sleeve to bind closely upon the core, or the core to bind closely within the sleeve, so as to diminish to, or near the point of elimination, any space whatever between the contacting surfaces. Even though in the bringing of the blank to rolling temperature, the higher coefficient of expansion of copper will tend to the creation of a space between the adjacent surfaces, nevertheless the step in the practice which I have now described as my invention, tending as it does to the opposite effect, will either wholly overcome, or reduce to a minimum, the tendency to separation.

I have in the foregoing passage described one manner of bringing the components together in which my invention may be practised. Another mode of assembling is this: One method of forming copper tubes which is now commercially practised is to shape the tube from a block of copper by the cooperating action of a perforating mandrel and shaping rolls. The copper, when undergoing this operation, is at relatively high temperature, though at a temperature lower than the melting point of copper. Instead of shaping such a tube upon a mandrel subsequently to be withdrawn, I may shape the tube upon the core of steel which remaining

in, forms one of the components of the finished article, and in this case by employing the core of steel at relatively low temperature, my invention may be enjoyed as will be understood from the foregoing description. 70

Still another method of forming copper tubes is what is known as the "extrusion method" in which a body of copper, heated to a point lower than the melting point of copper, is forced by pressure through an orifice, in which orifice is a central die or mandrel, a tube of copper being in this operation forced out through the orifice. I may practise my invention by having the tube, as it is extruded from the forming machine, pass over and surround a core of relatively cold steel, and in this case also it will be understood that the characteristic feature of my invention will be employed. In each of these cases it will be understood that the benefits of my innovation of operation will be realized when it comes to the heating and extending operation. 80

After the blank has been assembled by any one of the three ways which I have described, or in any other alternative way, the ends of it may, if desired, be painted or coated with a preparation of silicate of soda and ground asbestos, according to the practice now in use. Such coating is intended as a further safeguard against the ingress of air while the blank is under treatment. 90

While I have up to this point been careful to describe my invention as applicable to the production of a definite article, namely, copper-clad steel wire, it will be understood that it is broadly applicable to the production of articles compounded of other materials than copper and steel, and to articles of other form than that of wire, that is to say, it is broadly applicable to the forming of compound metallic articles produced by forging and reducing operations from blanks in which one body of metal increases another 105 body of metal. 110

To the essential portion of my process of preparation of the blank which I have now described, I may add another step, and this step consists in providing surfaces of contact between steel and copper at or near the opposite ends of the blanks as a whole, these surfaces of contact being so arranged and disposed that further treatment of the article after it has been assembled will in consequence of the difference in thermal expansion of the component bodies in a longitudinal direction effect a binding engagement of surface upon surface, to form a more effective seal against the ingress of or circulation 12 of air in any seam or gap between the copper and the steel. In this respect my invention is illustrated in the accompanying drawings. 115

Figure 1 is a view in longitudinal section 13

and elevation of the assembled blank; Fig. 2 is a view of like nature on a larger scale than Fig. 1 of a portion of the assembled blank, illustrating more clearly and somewhat diagrammatically the matter of the seal referred to; and Fig. 3 is a view similar to Fig. 2, illustrating a minor modification. 5

In the several figures corresponding parts bear the same numerals.

10 The steel core of the blank is indicated at 1 (1<sup>a</sup>), the copper sleeve at 2 (2<sup>a</sup>).

Referring first to Fig. 1, it will be seen that the steel core is made somewhat longer than the copper sleeve, and that near its opposite ends and at proper positions are cut V-shaped circumferential grooves. Into these V-shaped circumferential grooves the edges of the copper tube are shown to be turned. The turning in of the edges of the 20 copper tube in this manner may be effected by peening or spinning or otherwise.

In Fig. 3 the alternative consists in effecting an end to end contact of steel with copper not by turning the copper into a groove 25 in the steel, but by upsetting the ends of the slightly protruding core against the ends (shown to be properly beveled) of the copper sleeve.

Returning now to the operation already 30 described, let it be understood that a steel core of proper length and provided with grooves such as are illustrated in Fig. 1, and while cool, be introduced within a heated copper sleeve 2, and let it be understood that 35 the assembled parts have thereafter been brought to atmospheric temperature. The copper sleeve will then lie closely upon the steel core. At this stage of the operation the edges of the copper sleeve are peened or 40 spun into the previously formed grooves in the steel core so that the assembled blank will then appear as it is illustrated at Fig. 1. Thereafter, and in the further progress of 45 the operation already described, in consequence of the greater coefficient of expansion of copper, there will be a binding engagement longitudinally of surface upon surface, the edges of the copper sleeve binding against the outer walls of the grooves into 50 which it has been shaped, thus affording a seal against the ingress or circulation of air, either in such minute space as may exist between the component metals while in blank form, or in such small gaps as may form 55 themselves when the article is under treatment in the rolling mill. These surfaces of contact are indicated at *a*, *a* in Figs. 1 and 2. Like surfaces of contact, indicated by the letter *b*, exist in the case of Fig. 3, the contact having in this case been effected by the up-setting of the ends of the steel core; and the effect is the same, namely, that, by virtue of the relatively greater coefficient of expansion of copper, the contact effected at *b* is 60 made more effective by compression. The

seal so effected over transversely disposed contacting surfaces may, if desired, be made the more impervious, by the application to the surfaces of contact at the time they are shaped to engage one another, of a preparation of silicate of soda or other refractory fluid. Such an application of a third body is indicated in Fig. 2. 70

I claim herein as my invention:

1. The method herein described of forming compound metallic articles, which consists in applying to a body of metal while the said body is in solid state, and at relatively low temperature, an enveloping body of metal also in solid state but at a relatively high temperature; allowing an equalization in the temperature of the blank so compounded; and subjecting the compound blank to a reducing operation. 75

2. The herein described method of forming compound metallic articles which consists in applying to a core of steel in solid state, and at relatively low temperature, a sleeve of copper in solid state at relatively high temperature; allowing the temperature 80 of the blank so compounded to become equalized throughout; and subjecting the blank so compounded to a reducing operation. 90

3. The method herein described of forming compound metallic articles, which consists in shaping upon a body of metal in solid state and at relatively low temperature, an enveloping body of metal also in solid state, but at relatively high temperature; allowing an equalization of the temperature 95 of the blank so compounded, and subjecting the compound blank to a reducing operation. 100

4. The method herein described of forming compound metallic articles which consists in shaping upon a body of metal while 105 in solid state and at relatively low temperature, an enveloping body of metal also in solid state but at relatively high temperature; bringing the compound blank so formed to a temperature suitable for working and uniform throughout, and reducing the compound blank so heated. 110

5. The herein described method of forming compound metallic articles which consists in applying to a body of metal while 115 the said body is in solid state and at relatively low temperature, an enveloping body of metal also in solid state but at relatively high temperature, bringing the blank so compounded to a uniform temperature throughout, and a temperature suitable for forging, and then elongating the blank so compounded by forging. 120

6. The herein described method of forming compound metallic articles which consists in applying to a body of metal of relatively low coefficient of expansion while said body is in solid state and at relatively low temperature, an enveloping body of relatively high coefficient of expansion also in 130

solid state, but at relatively high temperature, allowing an equalization in temperature of the blank so compounded and bringing portions of one of the two component bodies to contact with portions of the other body over surfaces which extend transversely to the general length of the blank so compounded; heating said compound blank; and subjecting it to a reducing operation.

10 7. The herein described method of forming compound metallic articles which consists in applying to a core of steel in solid state, and at relatively low temperature, a sleeve of copper in solid state and at relatively high temperature; allowing the temperature of the blank so compounded to become equalized throughout, shaping one of the two component bodies to contact with the other of the two bodies over surfaces extending transverse to the general length of the compound blank as a whole; heating said

compound blank; and subjecting it to a reducing operation.

8. The method herein described of forming compound metallic articles which consists in applying to a core of metal of relatively low coefficient of expansion an enveloping body of a metal of relatively high coefficient of expansion, and bringing portions of one of the two component bodies 30 into contact with portions of the other body over surfaces which extend transversely to the general length of the blank so compounded; heating such compound blank; and subjecting it to a reducing operation. 35

In testimony whereof I have hereunto set my hand.

CHARLES W. DAVIS.

Witnesses:

L. McGREW,  
RALPH V. WILCOX.